

Nov. 13, 1928.

1,691,309

W. S. SMITH ET AL

LOADED ELECTRIC CONDUCTOR

Filed Nov. 17, 1926

*Fig. 1.*



*Fig. 2.*



INVENTORS

W. S. SMITH,  
H. J. GARNETT, AND  
J. A. HOLDEN,

By their Attorneys

*Baldwin & Wright*

## UNITED STATES PATENT OFFICE.

WILLOUGHBY STATHAM SMITH, OF BENCHAMS, NEWTON POPPLEFORD; HENRY JOSEPH GARNETT, OF SEVENOAKS; AND JOHN ANCEL HOLDEN, OF GIDEA PARK, ENGLAND.

## LOADED ELECTRIC CONDUCTOR.

Application filed November 17, 1926, Serial No. 149,007, and in Great Britain September 25, 1926.

This invention relates to loaded conductors, and more particularly to conductors of the kind commonly employed in telegraphy and telephony, in which the loading is provided in the form of a wire or tape of magnetic material wound upon the conductor. Such conductors are usually subjected to a process of annealing after having been wound with the wire or tape in order that the required magnetic properties may be developed in the loading material.

We have found, however, that when a conductor has been "whipped" at very high speed with, say, a hard drawn loading wire or tape, the required magnetic properties are apt not to be developed by the subsequent annealing process owing to the fact that the said loading wire or tape tends to grip the conductor proper to an extent sufficient to leave itself in a more or less highly strained condition, even after annealing.

According to this invention a spacing wire or the like, made of a material whose fusing temperature is not greater than the temperature at which the annealing process is carried out, is laid under the loading wire or tape so that during the annealing process the spacing wire fuses and so relieves the tension of the loading material.

The metal or alloy forming the spacing wire or the like must be such as will, on fusing, not injure or embrittle the conductor proper, and a copper-silver alloy of the composition 60% silver and 40% copper has been found particularly suitable for the purpose. The diameter of the spacing wire may be varied to suit various requirements, though it has been found that two thousandths of an inch is suitable in most cases.

The spacing wire may conveniently be laid approximately in a straight line along the copper conductor and may be attached in a suitable manner at the beginning of each length, but this not essential. To prevent

the loading wire (or tape) from sticking to the spacing wire during annealing, a slight oxidized loading wire (or tape) is preferably used.

The invention is diagrammatically illustrated in the accompanying drawings, in which Figures 1 and 2 are respectively half sectional views of a loaded conductor before and after annealing. In the drawings *a* indicates the conductor and *b* the loading ma-

terial. Referring to Figure 1, the spacing wire is shown at *c* and around which is an area denoted by the letter *d*. Referring now to Figure 2, which shows the loaded conductor after passage through the furnace, the spacing wire no longer exists in the form shown in Figure 1, but has melted and diffused into the copper of the conductor *a* forming a thin film and leaving an air space *e* over the film. It will be noted that the area *c* in Figure 2 is less than the area *d* in Figure 1, with the result that a slight loosening takes place in the loading material.

It should be understood that the view of the conductor in Figure 2 shows it in an intermediate stage, i. e. immediately after heat treatment and before it has cooled. During cooling, the loading wire or material *b* will further contract until the area *c* no longer remains.

## What we claim is:—

1. A method for the manufacture of loaded conductors which require heat treatment to develop the required magnetic properties, which comprises laying a metal spacer fusible at a temperature not exceeding the temperature for annealing the loading upon the conductor, winding the loading material over the conductor and the metal spacer and subjecting the loaded conductor to the said heat treatment which causes the metal spacer to melt.

2. A method for the manufacture of loaded conductors which require heat treatment to develop the required magnetic properties, which comprises laying a metal spacer composed of a silver-copper alloy and fusible at a temperature not exceeding the temperature for annealing the loading upon the conductor, winding the loading material over the conductor and the metal spacer and subjecting the loaded conductor to the said heat treatment which causes the metal spacer to melt.

3. A method for the manufacture of loaded conductors which require heat treatment to develop the required magnetic properties, which comprises laying a metal spacer composed of a silver-copper alloy containing 60% silver and 40% copper and fusible at a temperature not exceeding the temperature for annealing the loading upon the conductor, winding the loading material over the conductor and the metal spacer and subject-

ing the loaded conductor to the said heat treatment which causes the metal spacer to melt.

4. A method for the manufacture of loaded conductors which require heat treatment to develop the required magnetic properties, which comprises laying a metal spacer fusible at a temperature not exceeding the temperature for annealing the loading upon the conductor in an approximately straight line, winding the loading material over the conductor and the metal spacer and subjecting the loaded conductor to the said heat treatment which causes the metal spacer to melt.
5. A method for the manufacture of loaded conductors which require heat treatment to develop the required magnetic properties, which comprises laying a metal spacer 1/2000ths of an inch thick and fusible at a temperature not exceeding the temperature for annealing the loading upon the conductor, winding the loading material over the conductor and the metal spacer and subjecting the loaded conductor to the said heat treatment which causes the metal spacer to melt.

6. A method for the manufacture of loaded conductors which require heat treatment

to develop the required magnetic properties, which comprises laying a metal spacer fusible at a temperature not exceeding the temperature for annealing the loading upon the conductor, winding a superficially oxidized loading material over the conductor and the metal spacer and subjecting the loaded conductor to the said heat treatment which causes the metal spacer to melt

7. A method for the manufacture of loaded copper conductors which require heat treatment to develop the required magnetic properties, which comprises laying a metal spacer composed of a silver-copper alloy and fusible at a temperature not exceeding the temperature for annealing the loading upon the conductor, winding the loading material over the conductor and the metal spacer, and subjecting the loaded conductor to the said heat treatment, which causes the metal spacer to melt.

In testimony that we claim the foregoing as our invention, we have signed our names this 29th day of October, 1926.

WILLOUGHBY STATHAM SMITH.

HENRY JOSEPH GARNETT.

JOHN ANCEL HOLDEN.